

## UNITED STATES PATENT OFFICE

2,085,830

## MAGNETIC MATERIAL AND VANADIUM PENTOXIDE BONDING MEANS THEREFOR

Samuel Ruben, New Rochelle, N. Y.

No Drawing. Application March 6, 1936,  
Serial No. 67,491

4 Claims. (CL 175—21)

This invention relates to pressed and bonded granular materials, useful in the production of magnets.

An object of the invention is the provision of an improved bonding agent for magnets of the pressed type.

Another object is to provide a means whereby magnets may be simply and economically produced.

10 Further objects will be apparent from the disclosure.

It is desirable, in the provision of permanent magnet material, to have a bonding agent which will adhere as a very thin surface between the particles of the magnetic material and will allow the pressed and bonded material to be heat treated so as to provide maximum magnetic effects.

I have found that vanadium pentoxide is especially suitable for these purposes. It allows the production of a pressed magnet of the permanent type with materials ordinarily too brittle for practical use.

In the preparation of the material, the various elements entering into the composition of the magnet, for instance, nickel, aluminum, cobalt and iron, are processed into very finely divided granules and milled with powdered vanadium pentoxide in the proportion of about ten (10%) percent by weight of the magnetic material. In order to afford better contacting during the milling, a small amount of water can be added. The mixed mass is then pressed and heated to ap-

proximately 700° C. at which temperature the oxide flows and integrally combines with the surface of the granules, at the same time binding them together. When cooled, the material is a dense, tough structure with minimum gaps between the metal granules. It can be repeatedly heated or quenched without affecting its mechanical strength.

For a typical mixture, I may use twenty (20%) percent nickel, twenty (20%) percent aluminum, ten (10%) percent cobalt and fifty (50%) percent iron, these materials being combined with approximately ten (10%) percent of vanadium pentoxide. However, neither the materials themselves nor the percentages given are particularly critical—the invention being concerned chiefly with the use of vanadium pentoxide as a bonding material in magnets of the pressed or sintered type.

What is claimed is:

1. A magnet material comprising magnetic particles and vanadium pentoxide.

2. A magnet material comprising magnetic particles bound together by vanadium pentoxide.

3. A magnet comprising finely divided metal of the iron group bonded together by vanadium pentoxide.

4. The method of producing a magnet which comprises adding a quantity of vanadium pentoxide to particles of magnetic material compressing and heating the same until the vanadium pentoxide fluxes.

SAMUEL RUBEN.